

## UNITED STATES PATENT OFFICE.

WILLIAM BENJAMIN GERO, OF EAST ORANGE, NEW JERSEY, ASSIGNOR TO WESTINGHOUSE LAMP COMPANY, A CORPORATION OF PENNSYLVANIA.

## METHOD OF ALLOYING RARE METALS AND ARTICLES MADE THEREFROM.

No Drawing.

Application filed June 14, 1923. Serial No. 645,395.

To all whom it may concern:

Be it known that I, WILLIAM BENJAMIN GERO, a citizen of the United States, and a resident of East Orange, in the county of

5 Essex and State of New Jersey, have invented a new and useful Improvement in Methods of Alloying Rare Metals and Articles Made Therefrom, of which the following is a specification.

10 This invention relates to a process of alloying metals whereby corrosion from exposure may be prevented and more particularly to facilitate alloying of the rarer metals.

15 It is an object of the invention to provide a method of preparing easily corrodible metals so as to practically prevent corrosion preparatory to or during the alloying process.

20 It is a further object to provide a method whereby the constituent metals of the desired alloy may be more easily alloyed together.

25 Another object is to provide a method of alloying easily-oxidizable metals of the rare metal groups that will be readily applicable, efficient and have no deleterious effect upon the resultant product.

30 Further objects will become apparent from the description and claims.

It is desirable for all practical purposes, to prepare alloys of the rarer metals from their granular or powdered form owing to the susceptibility of such metals to corrosion.

35 while being heated to the extremely high temperatures at which the metals melt and to the impracticability of maintaining furnaces at the temperatures needed to melt the solid metals from mass form.

40 The rare metal alloys are usually prepared in slug form by compressing the mixed powders, firing and sintering. This process either necessitates the use of some suitable compound of the metal such as the oxide, to

45 which must be added a reducing agent before the metal itself is obtained, or, the metal must be used in powdered form, in which case corrosion by exposure to the ele-

ments before or during firing or sintering often takes place. Sintering in a vacuum 50 furnace may be necessary to prevent oxidation.

Certain metals of the group commonly known as rare or refractory metals, such as, uranium, zirconium, tungsten, etc., are peculiarly susceptible to corrosion when exposed to certain elements while in a finely divided state. If, however, the powders of the metals be consolidated into a coherent state, as by firing or sintering, corrosion is 60 effectively prevented. I do not attempt to explain this phenomenon but have found it to be as set forth.

The invention obviates corrosion of the metals, when in the powdered or granular state, by providing an individual impervious coating for each microscopic grain of the metal and a coating that will not only prevent corrosion for an indefinite period prior to firing and sintering, but also through the 70 critical stages of such treatment. There will be no objectionable débris left in the metal alloy, which will be wholly pure, as the coating will have been completely volatilized and expelled from between the metal particles prior to their thorough fusion. There

75 will result a non-porous and comparatively non-fragile bar of metal or metal alloy, if such be the original form of the product. The coating may be composed of any gum, 80 wax, resin or like substance, soluble in a suitable solvent, both of which substance and solvent, are completely volatile or leave no harmful residue in the desired metal or alloy.

85 In some cases it may be desirable or preferable to use paraffin with a solvent such as ether, a solution of the two being prepared in suitable proportions and the metal powders added in proportion to the quality and kind of alloy to be prepared. I have found that an excellent solution for the purpose may be prepared by dissolving paraffin in ether in the proportion of 0.12 gram of paraffin to 1 c. c. of ether, which may be 90 kept as a stock solution.

In preparing a tungsten-uranium alloy, for instance, I use that proportion of paraffin-ether solution which will thinly but thoroughly coat all grains of the tungsten and uranium powders. This proportion may be determined by calculation or experiment as will be readily understood. Sufficient of this stock solution of paraffin-ether is mixed with alcohol to give a percentage of paraffin to the 5 total weight of metal used, (e. g., tungsten and uranium) of from 0.1% to 1.5% by weight, depending upon the fineness and the amount of uranium used. The uranium or other similar metal is first mixed with alcohol, then with the solution containing the 10 paraffin. To this mixture is added the tungsten powder, slowly and in small portions, with continual stirring until all has been 15 added.

While it is desirable not to have an excess of the paraffin-ether solution, sufficient should be used to ensure a perfect mixture. The ether and alcohol may then be evaporated 20 from the mixture leaving the paraffin-coated metal intimately coagulated in a compound mixed form.

The coagulated mass thus formed may be 25 pressed into slugs of any desired density and sintered in any desirable manner to form metal bars or slugs for any purpose adaptable. During heating, the paraffin is 30 volatilized and driven off leaving an intimate mixture of the fine metal particles. If this process be used for alloying two or 35 more metals, an intimate diffusion of one through the other or others takes place and a true solid solution results.

The slugs may be sintered in a vacuum 40 furnace or other inert environment to insure that there will be no oxidation of the metals during heat treatment.

It will be noted that all of the ingredients 45 are protected against oxidation or corrosion throughout the complete process of mixing the metals in powdered form, compressing the powdered metals into slugs and in the sintering thereof into coherent bars.

Moreover, by introducing the powdered 50 metals into a wet solution, a more perfect mixture thereof can be obtained than by mechanically mixing the dry powders. The constituent metals are brought into an intimate association and when the paraffin and solvent are driven off by volatilization 55 a cleansing action of the metal powders takes place under certain conditions. Each of these results greatly assists alloying.

The method has been described with 60 particular reference to an alloy of two or more of the rare or refractory metal groups but as it may be readily practiced to alloy a rare or refractory metal with one of the common or baser metals, it is not desired 65 that the process be limited except by the scope of the claims appended.

What is claimed is:

1. The steps in the method of preparing a refractory metal from a comminuted form which comprise, coating the individual particles thereof with a volatile protective agent and sintering said particles into a coherent state. 70
2. The steps in a method of making an alloy with a refractory metal which comprise, comminuting the constituent metals 75 in a finely divided form, pressing the comminuted metals into a slug and protecting said refractory metal from exposure to the elements during such operation by a protective covering intimate therewith. 80
3. The method of preparing refractory metals which consists in coating a powdered metal with a volatile protective material, pressing the coated metal powder into a slug and sintering the slug into a coherent 85 body. 85
4. The method of preparing refractory metals which consists in coating a powdered metal with a volatile protective material, pressing the coated metal powder into a 90 slug and sintering the slug into a coherent body in an inert environment. 90
5. The method of protecting powdered refractory metal from contamination during fabrication thereof into a coherent body 95 which consists in coating the metal powder with a volatile protective material and sintering the coated metal powder into a compact body in an inert environment. 95
6. The method of making coherent refractory bodies consisting in coating a powdered refractory metal with a solid protective coating, pressing the coated metal into a slug and sintering in an environment inert with respect thereto. 100 100
7. The method of making alloys of refractory metals consisting in mixing the alloying metals in powdered form in a solution containing a volatile constituent, evaporating the solvent to produce a coating of the volatile constituent on the powdered metals, conglomerating the metals and sintering. 110 110
8. The method of making coherent refractory metal bodies consisting in coating the metal in powdered form with paraffin, pressing the coated metal into a slug and sintering in an environment inert with respect to the metal. 115
9. The method of protecting powdered refractory metal during fabrication into coherent bodies consisting in coating the powdered metal with a volatile material impervious to the atmosphere and heat treating said metal in an environment inert with respect thereto to volatilize out said coating material and sinter the metal into a coherent form. 120 125
10. The method of protecting powdered refractory metals from corrosion consisting 130

in introducing the powdered metal into a solution of a corrosion proofing material and dissolving the solvent from said solution to coat the metal powder with the corrosion proofing material.

11. The method of preparing refractory metal powders for alloying comprising, in part, mixing the individual grains of the

constituent powders in a solution containing a soluble material solid at ordinary temperatures, and volatilizing the solvent to coat the powders with the solid constituent.

In testimony whereof, I have hereunto subscribed my name this 13th day of June, 1923.

WILLIAM BENJAMIN GERO.